

# United States Patent Office

NATHANIEL IRISH, OF ROCHESTER, MINNESOTA.

Letters Patent No. 84,421, dated November 24, 1868.

## IMPROVED COMPOUND FOR ROOFING AND PAINTING.

The Schedule referred to in these Letters Patent and making part of the same.

To all whom it may concern:

Be it known that I, NATHANIEL IRISH, of Rochester, in the county of Olmsted, and in the State of Minnesota, have invented certain new and useful Improvements in Compound for Roofing and Painting; and do hereby declare that the following is a full, clear, and exact description thereof.

My invention consists in mixing certain ingredients, hereinafter specified, to form a compound suitable for roofing, painting, and a variety of other purposes, so as to make the article to which it is applied perfectly impervious to water.

The ingredients used are, boiled linseed-oil, plaster of Paris, white or colored lead, Venice turpentine, and water.

For roofing, they are mixed in the following proportions: Ten pounds plaster of Paris, one gallon water, and a half pint boiled linseed-oil, to which add one-sixteenth part of lead, and, to one gallon of the mixture thus made, one ounce of Venice turpentine.

When, now, tempered to such a degree that it may be applied with a mason's trowel, it is far superior, for roofing-purposes, to any other compound now in use,

as it is perfectly impervious to water, and when it becomes dry, will not crack and scale off.

For painting, I take equal parts of lead and plaster Paris, with sufficient boiled linseed-oil to render it suitable for applying with brush, after which I may add the Venice turpentine.

I do not desire to confine myself to any exact proportion of these ingredients, as my invention embraces the art of mixing the above composition, both hard and soft, to suit the different uses to which it may be applied.

Having thus fully described my invention,

What I claim as new, and desire to secure by Letters Patent, is—

A compound, consisting of the above-mentioned ingredients, and used substantially as and for the purposes herein set forth.

In testimony that I claim the foregoing, I have hereunto set my hand, this 21st day of September, 1868.

NATHANIEL IRISH.

Witnesses:

J. V. DANIELS,  
CHAS. SHANDREW.